

R. FRIESE.

INSULATOR.

APPLICATION FILED JAN. 7, 1911.

1,107,281.

Patented Aug. 18, 1914.



Fig. 4



Fig. 5



WITNESSES

H. H. King

Emmanuel M. Lenster

INVENTOR

Robert Friese  
By his attorneys  
Stone & Woodward

# UNITED STATES PATENT OFFICE.

ROBERT FRIESE, OF CHARLOTTENBURG, GERMANY, ASSIGNOR TO SIEMENS-SCHUCKERT-WERKE G. M. B. H., OF BERLIN, GERMANY, A CORPORATION OF GERMANY.

## INSULATOR.

1,107,281.

Specification of Letters Patent. Patented Aug. 18, 1914.

Application filed January 7, 1911. Serial No. 601,435.

*To all whom it may concern:*

Be it known that I, ROBERT FRIESE, a subject of the German Emperor, and residing at Charlottenburg, near Berlin, Germany, **5** have invented certain new and useful Improvements in Insulators, of which the following is a specification.

My invention relates to insulators having the action of condensers.

**10** Condensers and leading-in insulators are known containing in the dielectric electrically conducting intermediate layers which gradually decrease in length as they are farther from the center, for the purpose of **15** distributing the strength of the electric field so that the dielectric is subjected to a more favorable stress and the insulation is consequently utilized better.

Sheet metal or foil has been used heretofore for the electrically conducting intermediate layers which were built up a layer at a time to form the condenser or the like. This mode of manufacture was however not suitable for many purposes. A leading-in **25** insulator such as will be described herein-after could be made according to this known method only by winding the electrically conducting intermediate layers.

**30** A primary object of my invention is to provide not only an easier and cheaper mode of manufacturing such insulators having the action of condensers, but also improved condensers, insulators and the like of the type described.

**35** Some illustrative embodiments of my invention are represented by way of example in the accompanying drawing, wherein:—

Figures 1 and 2 show parts of a condenser in cross-section and longitudinal section, **40** respectively; Figs. 3 and 4 are longitudinal section and cross-section, respectively, showing a leading-in insulator having the action of a condenser, and Fig. 5 is a section showing a condenser comprising electrically conducting intermediate layers not extending to the outside of the same.

Referring to the drawing,  $b_1$  designates the outer coating,  $b_2$  the inner coating,  $s_1$ ,  $s_2$  . . . electrically conducting layers, and **45**  $d_1$ ,  $d_2$  . . . the dielectric of the condensers or leading-in insulators for high tensions.

In condensers and leading-in insulators as shown in Figs. 3 and 4 there is the danger that as the tension increases sparks will pass **50** between the points  $s_1$  and  $s_2$ . This danger is

particularly great when the insulators are employed at places where the surface of the dielectric is subjected to the influence of the weather or moisture.

According to my invention, in order to **60** prevent the insulators being ruptured by the high tension I do not allow the electrically conducting intermediate layers to extend quite to the surface of the dielectric, as clearly shown in Fig. 5. Further, it has **65** been found that the electrically conducting intermediate layers serve their purpose even when they possess very little conductivity. On the one hand, the displacement currents which are equalized in the intermediate layers are only to be estimated in milliamperes **70** even in large apparatuses, for example large leading-in insulators, as calculation and observations have shown. But as, on the other hand, the differences of potential between **75** the coatings of individual condensers may be several thousand volts, it will be readily understood that the intermediate layers frequently require to possess only such small conductivity that in other spheres of em- **80** ployment they would in practice be looked upon as insulators. Electrically conducting intermediate layers of metal therefore generally require to be of only microscopic thickness. Making use of this circumstance, **85** leading-in insulators of the type represented in Figs. 3 and 4, for example, may be formed of concentric glass or porcelain tubes provided with a thin metallic deposit as coating. As spaces or gaps between the individual tubes cannot be avoided in such insulators I prefer to employ an electrically conducting material between the coatings, **90** e. g. tin-foil, powdered metal, powdered carbon and the like, which may be forced into the gaps or spaces between the coatings, so that after its insertion it forms a more or less solid conducting mass. Condensers, **95** insulators and other apparatus having the action of condensers not of tubular shape **100** can of course be made in a similar manner.

The above mentioned substances for electrically connecting adjacent coatings, particularly metallic powder and powdered carbon, may, when suitable, themselves form **105** electrically conducting intermediate layers, so that connecting coatings or coverings on the surfaces of the dielectric are unnecessary, because the grains which are close together and contact with the surfaces of the **110**

dielectric are to be looked upon more or less correctly as electrically conducting coatings. As the resistance of the electrically conducting intermediate layers may be very considerable without the layers ceasing to serve their purpose, they do not necessarily have to be composed of metal, but it is frequently preferable to make them of substances known briefly as bad conductors. It has been found, for example, that not only gypsum containing electrically conducting admixtures but gypsum itself without any special admixture of electrically conducting substances may be employed with complete success for the electrically conducting intermediate layers. Admixtures of powdered carbon or metallic powder and the like can be used to assure the small requisite conductivity of gypsum or cement, and particularly also certain salts, such as chlorid of sodium or chlorid of magnesium. Under certain circumstances solutions or liquid acids may also be employed. In general, on account of the but small requisite conductivity, the intermediate layers may be made of conductors of the second class with and without admixtures of conductors of the first class.

The condensers or insulators according to my invention may be shaped according to the circumstances in each case. It is only essential that the dielectric-layers which are not perfect non-conductors of electricity be separated by intermediate layers which in comparison with the former possess a materially greater conductivity, even if this be small in itself. These relations may briefly be stated by saying that the dielectric-layers must be separated by intermediate layers of only small conductivity.

Condensers of the type described possess special advantages with regard to the mode

by which they can be manufactured. For example, they can be made by employing as the material either for the dielectric or for the conducting intermediate layer a liquid, or a substance which softens when heated. If such a substance be used for the dielectric, the plastic or liquid dielectric can be poured or pressed into the rigid, electrically conducting intermediate layers, where it will solidify while if such a substance be used for the intermediate layers it can be poured into suitable cavities in the rigid dielectric. Either the intermediate layers or the layers of the dielectric consequently form, during the manufacturing operation, a rigid body having spaces or chambers into which the material composing the dielectric or that composing the electrically conducting intermediate layers is inserted in mobile condition such as powdered, pasty, liquid or the like, this material being adapted to subsequently solidify. This mode of manufacturing such condensers or the like has, in addition, the advantage that spaces containing air in the interior of the condensers or the like can be completely avoided.

I claim:

As a new article of manufacture, an insulator having the action of a condenser, comprising a plurality of layers of a solid dielectric of varying lateral extension, alternating with a plurality of layers of a plastic material of small electric conductivity adapted to solidify between said dielectric layers.

In testimony whereof I have signed my name to this specification in the presence of two witnesses.

ROBERT FRIESE.

Witnesses:

HENRY HASPER,  
WOLDEMAR HAUPP.